

# UNITED STATES PATENT OFFICE.

JOHANNES ANDERSEN, OF LILLEHAMMER, NORWAY.

## INSULATING MASS ESPECIALLY FOR ELECTRIC USE.

1,285,889.

Specification of Letters Patent. Patented Nov. 26, 1918.

No Drawing.

Application filed June 1, 1916. Serial No. 101,111.

To all whom it may concern:

Be it known that I, JOHANNES ANDERSEN, citizen of Norway, residing at Lillehammer, Norway, have invented new and useful Improvements in an Insulating Mass Especially for Electric Use, of which the following is a specification.

My invention relates to insulating compositions more particularly intended for electrical purposes.

Electric insulating masses or compositions as hitherto used are objectionable in many respects.

The usually employed composition is expensive and when hardened is rather brittle at low temperatures, so that it easily fractures. When exposed to heat it becomes plastic, and is therefore generally warmed before it is placed in position. This property, however, is frequently detrimental because the heat of the sun is sufficient to make the mass plastic to such a degree that it gets out of shape, and if subjected to greater heat, as may easily happen in many electric plants, the mass may completely melt and run off.

My invention has for its object to produce an insulating mass which is free from the defects above referred to. Its principal constituent is Norwegian steatite (talc) or soapstone in a more or less pulverized state held together by a suitable binder.

The binder may be varied and may consist of resin and linseed oil, of shellac or the like.

The principal constituent, the Norwegian steatite (talc) ("klæbersten") is, among the Norwegian natural stones, the kind which is least affected by acids and by direct heat. Furthermore it has great resistance to rapid variations of temperature and is very effective for insulating electric currents.

It therefore is an efficient electric insulator.

As an example of a good insulating composition the following proportions may be employed.

|                        |     |
|------------------------|-----|
| Steatite (talc) powder | 50% |
| Resin                  | 40% |
| Linseed oil            | 10% |

The linseed oil is first somewhat concentrated, by boiling, and then the resin is added. When these two substances have been well boiled together, the steatite (talc)

powder is stirred in. After cooling the mass is kneaded, whereby it acquires great elasticity.

The resin is undoubtedly in itself an insulator, but in the present case it is used essentially as a binder. When boiled together with linseed oil the mass becomes plastic, and after the addition of the powder it has a certain degree of elasticity.

In addition to being considerably cheaper than known insulating compounds my composition does not melt in boxes, into which it is filled for the purpose of serving as an insulator and will therefore not run off. Even if the binder should burn, the steatite (talc) remains around the cables, etc., in a pulverized state, so that it still acts as an insulator.

As the mass is very elastic, it need not be heated before being used, for instance, as an insulation for conductors. A thin disk may be cut off, which is kneaded for a few moments between the fingers, when the mass on account of its elasticity can be easily placed upon any cable.

The mass has a heat extension coefficient which is practically zero. Moreover there is no trace of hygroscopicity.

An example of the use of shellac as a binder is as follows:

|                 |     |
|-----------------|-----|
| Steatite (talc) | 50% |
| Shellac         | 20% |

and some drops of alcohol for dissolving the shellac. This mass possesses about the same properties as that first described.

I claim as my invention:

An insulating composition comprising powdered steatite (talc) and a mixture of resin and linseed oil in about the following proportions:

|                 |     |
|-----------------|-----|
| Steatite (talc) | 50% |
| Resin           | 40% |
| Linseed oil     | 10% |

In testimony whereof I have signed my name to this specification in the presence of two subscribing witnesses.

JOHANNES ANDERSEN.

Witnesses:

AXEL LAHN,  
MAGENS BUGGE.